

## UNITED STATES PATENT OFFICE

2,361,051

## LUBRICANT

John A. Patterson and Rush F. McCleary, Beacon, N. Y., assignors to The Texas Company, New York, N. Y., a corporation of Delaware

No Drawing. Application March 31, 1942,  
Serial No. 436,968

13 Claims. (Cl. 252—48)

This invention relates to the use of metal derivatives of sulfurized compositions obtained or derived from cashew nut shell oil in hydrocarbon oils, particularly petroleum oils, to improve the properties of lubricants compounded therewith.

It is generally recognized that the recent developments in the automotive industry directed toward the increase in power output and efficiency of mechanical equipment have set up such severe and exacting operating conditions as to necessitate an improvement in the highly refined hydrocarbon oils used in the lubricating system thereof. Thus the increase in operating temperatures and engine speeds, together with reduced clearances between the moving parts and the use of hard-bearing alloys such as copper-lead, cadmium-silver, etc. have seriously accentuated such problems as corrosion, oxidation and varnish and lacquer formation with the resultant deleterious effect on the efficiency of the equipment. Previous attempts have been made to eliminate these deficiencies in the lubricants by incorporating in the highly refined hydrocarbon oils proportions of additive ingredients possessing inhibiting properties.

The natural occurring cashew nut shell oil is described in Matiello, J. J., "Protective & Decorative Coatings," Chap. 2 (1941), as containing approximately 90% anacardic acid ( $C_{22}H_{32}O_3$ ) and 10% cardol ( $C_{32}H_{52}O_4$ ) when extracted from the shells by means of solvents. This composition is very unstable and is subject to polymerization, condensation and decomposition on heating.

The usual commercial methods of extracting the oil from the cashew nut shells are incidental to the extraction of the kernel. The cellular structure of the shell is destroyed by a thermal treatment such as a charring or carbonizing process which expels the oil and facilitates removal of the kernel. The extracted shell oil is collected as a dark, thick, viscous liquid whose chemical composition varies in accordance with the degree of heat used in the extraction process.

These thermally extracted oils are described as consisting primarily of anacardic acid, cardanol ( $C_{20}H_{32}O$ ) and cardol with cardanol predominating. The particular proportions of these components vary in accordance with the amount of heat used in the extraction process as, for example, when extracting at low temperatures of approximately 400° F., the extracted oil contains approximately 70% cardanol, whereas extracting at roasting temperatures yields an oil containing approximately 40-50% cardanol.

It has been discovered that the addition of a

small quantity of an oil-soluble or oil-miscible metal derivative of sulfurized cardanol to a refined hydrocarbon oil provides a lubricant or a compounding lubricant which possesses improved detergent and anti-oxidant or anti-corrosive properties.

The refined hydrocarbon oils which may be improved by the compositions of the present invention include the petroleum lubricating oils used as motor, Diesel, turbine and aviation oil and the hydrocarbon oils used in the preparation of industrial lubricants, greases, textile oils, etc.

Distillation of the commercial cashew nut shell oil carried out either at greatly reduced pressure or steam distillation at atmospheric pressure yields a distillate consisting almost entirely of cardanol. Cardanol distills over as a light colored liquid at approximately 225° C. and 10 mm. mercury. This compound is described as a phenol derivative possessing an unsaturated alkyl radical in the meta position. This compound is very unstable and upon heating forms condensation and polymerization products, together with copolymers. In addition to the cardanol, the distillate obtained contains a lower boiling fraction possessing a nicotine-like odor which rapidly darkens when exposed to the atmosphere. This fraction which amounts to about 5% of the original oil contains approximately 0.64% nitrogen. If desired, this lower boiling fraction may be removed by fractional distillation.

Another method of obtaining cardanol is the destructive distillation of the solvent extracted cashew nut shell oil. The yields obtained will vary according to the degree of decomposition of the solvent extracted oil. The following physical constants were obtained on two distillates of the commercially available thermal extracted cashew nut shell oil, one being obtained by vacuum distillation at 10 mm. Hg (A), and the other by steam distillation at atmospheric pressure (B).

|                    | A    | B    |
|--------------------|------|------|
| 45 Bromine No.     | 135  | 118  |
| Hydroxyl No.       | 183  | 181  |
| Neutralization No. | 6    | 3.5  |
| Saponification No. |      | 8.4  |
| Per cent sulfur    | 0.10 | 0.10 |

50 The term "cardanol" as used throughout the specification and claims, unless otherwise stated, is meant to include not only the specific compound which has a constant boiling point at approximately 225° C. and 10 mm. Hg, but also the distillation products obtained by the distilla-

tion of the thermal extracted cashew nut shell oil at reduced pressures or by steam distillation at atmospheric or reduced pressure and the distillate obtained by the destructive distillation of the solvent extracted cashew nut shell oil.

The particular metals which may be used to form the oil-soluble metal derivatives of the present invention include any of the following metals: sodium, potassium, lithium, calcium, barium, strontium, tin, bismuth, aluminum, zinc, magnesium, cadmium, lead, titanium, antimony, chromium, manganese, iron, cobalt, nickel and copper, with preference given to the alkaline earth metals and tin and zinc.

These oil-soluble metal derivatives of the present invention may be incorporated in a hydrocarbon oil in amounts varying between 0.01 to 5.0% by weight of the finished lubricant. The particular proportions used depend upon the type of lubricant to be improved, the service for which the lubricant is intended, and the degree of improvement desired in the hydrocarbon oil. The preferred range of proportions in a mineral lubricating oil when used in a few of the more common services are as follows:

|                            | Per cent by weight of finished lubricant |
|----------------------------|------------------------------------------|
| Diesel lubricating oil     | 0.5 - 1.0                                |
| Motor lubricating oil      | 0.3 - 0.6                                |
| Heavy duty lubricating oil | 0.5 - 2.5                                |
| Turbine lubricating oil    | 0.01 - 0.1                               |
| Airplane lubricating oil   | 0.2 - 0.6                                |

When preparing the oil-soluble additive ingredients in the present invention, such methods and conditions of reaction must be chosen which will avoid the formation of polymerization and condensation products and insure the formation of an oil-soluble product. In the present instance it is preferable to first stabilize the cardanol by reducing the degree of unsaturation through partial hydrogenation. This may be done either prior to or simultaneously with the formation of the metal derivative or prior to the sulfurization reaction depending upon which sequence of reactions is used. This invention is not limited to these particular methods of preparation, and any other classical methods may be used together with any sequence of reactions which result in the formation of oil-soluble or oil-miscible metal derivatives of sulfurized cardanol.

If it is desired to prepare the metal derivative prior to sulfurization, the cardanol may be initially subjected to partial hydrogenation, such as hydrogenation with Raney nickel catalyst under pressure, or simultaneously hydrogenated during the neutralization reaction by reacting the cardanol with a solution of the desired metal in liquid ammonia. In the latter reaction the residual hydrogen displaced by the metal partially hydrogenates the unsaturated constituents.

If, on the other hand, the sulfurization reaction precedes the neutralization step, particular care must be taken to insure an oil-soluble product. In the usual reaction of sulfur with cardanol, polymerization products are obtained which range from semi-solid to solid rubbery materials which are oil-insoluble. This type of reaction is to be avoided since the metal derivatives of these types of compositions are usually also oil-insoluble. However, if prior to the sulfurization reaction the cardanol was partially hydrogenated, the tendency toward the formation of polymerization products is reduced to a minimum.

Although it is preferred to use the foregoing stabilizing reactions prior to sulfurization, other methods can be employed. One of these methods which avoids the hydrogenation step is the direct sulfurization with sulfur, at low temperatures, in the presence of solvent diluents such as lubricating oil, xylenes, etc. In every instance, the amount of sulfur which may be incorporated into the unsaturated constituents of cardanol will depend upon the degree of unsaturation.

The following examples illustrate two of the methods which might be used in preparing the foregoing types of compounds:

#### EXAMPLE I

An ethyl alcohol solution of 514 grams of distilled cashew nut shell oil of the distillate obtained from the distillation of commercially available cashew nut shell oil was charged in a hydrogenation bomb with 10-15 grams of Raney nickel catalyst and treated with hydrogen under pressure. The temperature was controlled by external heat and varied between 50° F. at the start to 200° F. near the end. The product, after being freed of catalyst and solvent, weighed 495 grams and had a bromine number of 80.

533 grams of the partially hydrogenated product was added to 84 grams of sulfur in 750 cc. 30 of xylene and stirred together. This mixture was then heated for seven hours at 140-150° F. To the resulting sulfurized product 175 grams of anhydrous barium hydroxide in 500 cc. of toluene were added. The mixture was heated to refluxing temperature under an automatic water separator until no more water was evolved. The slight excess of barium hydroxide was filtered out and the solvent was subsequently removed by distillation in vacuo. A sample of the resulting barium derivative analyzed 27.0% ash, 9.03% sulfur and 18.8% barium.

#### EXAMPLE II

415 grams of cardanol (bromine number 105) 45 was dissolved in twice its volume of toluene and added to a solution of 50 grams of technical calcium metal in three liters of liquid ammonia with vigorous agitation over a period of two hours. After the addition was complete, the ammonia was 50 allowed to boil off and the residual toluene solution filtered to remove excess calcium and other impurities. The solvent was removed by distillation in vacuo and the product converted to a 50% concentrate by dissolving it in an equal weight of lubricating oil. The concentrate analyzed 3.6% calcium and had a bromine number of 45. This corresponds to a decrease in unsaturation equivalent to the amount of hydrogen displaced by the calcium.

60 A mixture of 760 grams of a 25% concentrate of the calcium derivative of partially hydrogenated cardanol in lubricating oil, 16 grams of sulfur and 500 cc. of xylene were heated with stirring to 150° C. and maintained at that temperature for two hours. The xylene was subsequently removed by distillation in vacuo and the resulting 25% concentrate analyzed 1.86% calcium and 1.78% sulfur.

70 The effectiveness of the compositions of the present invention as improving agents for lubricants was demonstrated by empirical tests, together with tests in actual automotive engines. The following empirical test was designed to illustrate the anti-oxidant or anti-corrosive properties of the additive ingredient in a lubricating

oil. This test consists of a copper-lead bearing specimen encased in a special non-wearing bushing, rotatively mounted on a stainless steel shaft and immersed in a glass pot of the oil to be tested. Both fine structure and coarse structure copper-lead bearing specimens were used. The oil was heated to a controlled temperature of either 250° F. or 350° F. and continuously circulated between the bearing specimen and the shaft for 10 hours. Throughout the test the oil was continuously agitated by means of copper baffles which acted as oxidation accelerators. The bearing specimen was weighed before the test and after the 10-hour period and the loss of weight recorded in milligrams. The reference oil of this test was a solvent refined, dewaxed, Mid-Continent lubricating oil of an S. A. E. 30 grade. The following

## Reference oil

| Engine part                   | 120 hours                                                                      | 240 hours                                        |
|-------------------------------|--------------------------------------------------------------------------------|--------------------------------------------------|
| 5 Piston crown                | Normal                                                                         | Normal                                           |
| Scuffing above heat groove    | D                                                                              | C                                                |
| Heat groove                   | B                                                                              | D                                                |
| Ring grooves                  | A                                                                              | B                                                |
| Piston skirt                  | B                                                                              | B                                                |
| Under piston deposit          | A                                                                              | A                                                |
| Filter                        | A                                                                              | A                                                |
| Ring lands                    | A                                                                              | B                                                |
| Ring cleanliness              | #1, 2, 3, 6 clean; #4 lacquer on top; #5 trace lacquer on top. Oil holes open. | #1, 2, 3 clean; #4 lacquer; #5, 6 light lacquer. |
| Rings stuck                   | None                                                                           | None                                             |
| 15 Bearing weight loss, grams |                                                                                | 0.027.                                           |

## Reference oil plus 0.5% barium salt of sulfurized partially hydrogenated cardanol (Example I)

| Engine part                | 120 hours                                                                      | 240 hours                                        | 360 hours                                           | 480 hours                                     |
|----------------------------|--------------------------------------------------------------------------------|--------------------------------------------------|-----------------------------------------------------|-----------------------------------------------|
| Piston crown               | Normal                                                                         | Normal                                           | Normal                                              | Normal                                        |
| Scuffing above heat groove | D                                                                              | C                                                | C                                                   | C                                             |
| Heat groove                | B                                                                              | D                                                | D                                                   | D                                             |
| Ring grooves               | A                                                                              | B                                                | B                                                   | C                                             |
| Piston skirt               | B                                                                              | B                                                | B                                                   | B                                             |
| Under piston deposit       | A                                                                              | A                                                | A                                                   | B                                             |
| Filter                     | A                                                                              | A                                                | A                                                   | B                                             |
| Ring lands                 | A                                                                              | B                                                | B                                                   | B                                             |
| Ring cleanliness           | #1, 2, 3, 6 clean; #4 lacquer on top; #5 trace lacquer on top. Oil holes open. | #1, 2, 3 clean; #4 lacquer; #5, 6 light lacquer. | #1, 2, 3 clean; #4, 5 lacquer; #5, 6 light lacquer. | #1, 2, 3 clean; #4, 5 lacquer; #5, 6 varnish. |
| Rings stuck                | None                                                                           | None                                             | None                                                | None.                                         |
| Bearing weight loss, grams |                                                                                |                                                  | 0.030.                                              |                                               |

results were obtained on the uninhibited reference oil and the reference oil compounded with the additives of the present invention.

## Bearing corrosion—copper-lead (10 hours)

[Loss of weight, mgs.]

|                                                                                            | 250° F.      | 350° F.            |
|--------------------------------------------------------------------------------------------|--------------|--------------------|
| Reference oil                                                                              | 4-6<br>19-15 | 177-142<br>250-275 |
| Reference oil+0.5% barium salt of sulfurized partially hydrogenated cardanol (Example I)   | 0-0          | 47-76              |
| Reference oil+0.5% calcium salt of sulfurized partially hydrogenated cardanol (Example II) | 10           | 132                |

1 Coarse structure.

As a test to indicate the effectiveness of the additive ingredients of the present invention under actual operating conditions in an automotive engine, a special test was devised which is a modification of the test described in Diesel Lubricant Test Manual, Laboratory Test No. 1, issued by the Caterpillar Tractor Company. This test was carried out in a single cylinder Diesel engine operating at 900 R. P. M. with a water jacket temperature of 175° F. The test was run continuously for 480 hours at increments of 120 hours or until rings are stuck as indicated by the increase in blow-by. The crankcase oil was drained every sixty hours and fresh oil added thereto. At the end of each test period, the engine was thoroughly examined and any carbonaceous deposits, lacquer and sludge formation, etc. were noted and the principal engine parts classified according to their condition. In the present instance the reference oil was a mixed base solvent-refined, dewaxed Mid-Continent lubricating oil of an S. A. E. 30 grade. The results of the test runs on the reference oil and the reference oil containing 0.5% barium salt of sulfurized partially hydrogenated cardanol (Example I) are as follows:

| 35 | Engine part                | Rating           | Condition noted                                                                                                               |
|----|----------------------------|------------------|-------------------------------------------------------------------------------------------------------------------------------|
|    | Scuffing above heat groove | A<br>B<br>C<br>D | No scuffing to very fine scuffing.<br>Up to 50% scuffed.<br>Up to 75% scuffed.<br>Over 75% scuffed.                           |
| 40 | Heat groove                | A<br>B<br>C<br>D | Open to 10% plugged.<br>Up to 50% plugged.<br>Up to 75% plugged.<br>Over 75% plugged.                                         |
|    | Ring groove                | A<br>B<br>C      | Clean to heavy lacquer.<br>Slight carbon in Nos. 1 and 2.<br>Heavier deposits.                                                |
| 45 | Piston skirt               | A<br>B<br>C<br>D | Clean to very slight trace of varnish.<br>Trace varnish to light varnish.<br>Heavy varnish to lacquer.<br>Very heavy lacquer. |
|    | Under piston deposit       | A<br>B<br>C      | Clean to discoloration.<br>Trace deposit.<br>Heavy deposit.                                                                   |
| 50 | Filter                     | A<br>B<br>C      | Clean to mesh pattern visible.<br>Mesh pattern visible to slight amount mud sludge.<br>Heavy mud or carbonaceous deposit.     |
|    | Ring land                  | A<br>B           | Clean to heavy varnish.<br>Heavy varnish to carbon deposit.                                                                   |

55 The hydrocarbon oils to which the oil-soluble metal derivatives of the present invention are added may be either in the crude form or partially or highly refined and may contain other additive ingredients such as dyes, metal soaps, 60 pour depressants, thickeners, V. I. improvers, oiliness agents, extreme pressure agents, sludge dispersers, oxidation inhibitors, and corrosion inhibitors such as sulfurized hydrocarbons, etc.

Obviously many modifications and variations 65 of the invention, as hereinbefore set forth, may be made without departing from the spirit and scope thereof and, therefore, only such limitations should be imposed as are indicated in the appended claims.

70 We claim:

1. A lubricant comprising a hydrocarbon oil and a small quantity, less than 5.0% by weight, of an oil-soluble metal derivative of sulfurized partially hydrogenated cardanol.
2. A lubricant comprising a mineral lubricat-

ing oil and 0.01-5.0% by weight of an oil-soluble metal derivative of sulfurized partially hydrogenated cardanol.

3. A lubricant comprising a mineral lubricating oil and 0.01-5.0% by weight of an oil-soluble alkaline earth metal derivative of sulfurized cardanol.

4. A lubricant comprising a mineral lubricating oil and 0.01-5.0% by weight of an oil-soluble alkaline earth metal derivative of sulfurized, partially hydrogenated cardanol.

5. A lubricant comprising a hydrocarbon oil having incorporated therein 0.01-5.0% by weight of an oil-soluble metal derivative of sulfurized cardanol.

6. A lubricant comprising a hydrocarbon oil having incorporated therein 0.01-5.0% by weight of an oil-soluble metal derivative of sulfurized partially hydrogenated cardanol.

7. A lubricant comprising a hydrocarbon oil and 0.01-5.0% by weight of an oil-soluble alkaline earth metal derivative of sulfurized cardanol.

8. A lubricant comprising a hydrocarbon oil and 0.01-5.0% by weight of an oil-soluble alkaline earth metal derivative of sulfurized partially hydrogenated cardanol.

9. A lubricant comprising a mineral lubricating oil and 0.01-5.0% by weight of a tin derivative of sulfurized cardanol.

10. A lubricant comprising a mineral lubricating oil and 0.01-5.0% by weight of a tin derivative of sulfurized partially hydrogenated cardanol.

11. A lubricant comprising a mineral lubricating oil and 0.01-5.0% by weight of a zinc derivative of sulfurized cardanol.

12. A lubricant comprising a mineral lubricating oil and 0.01-5.0% by weight of a zinc derivative of sulfurized partially hydrogenated cardanol.

13. A lubricant comprising a hydrocarbon oil and a small quantity of an oil-soluble metal derivative of sulfurized cardanol, said quantity being sufficient to impart anti-oxidant properties to said hydrocarbon oil constituent.

JOHN A. PATTERSON.  
RUSH F. McCLEARY.